

# UNITED STATES PATENT OFFICE.

ROGER BUCHANAN COCK, OF GOMSHALL, ENGLAND, ASSIGNOR TO HIMSELF AND WILLIAM WILLOUGHBY WILLIAMS, OF "BODELWYDDAN," RHYDDLAN, FLINT, ENGLAND.

## TANNING COMPOSITION.

1,402,283.

Specification of Letters Patent.

Patented Jan. 3, 1922.

No Drawing.

Application filed October 31, 1918. Serial No. 260,562.

To all whom it may concern:

Be it known that I, ROGER BUCHANAN COCK, subject of the King of Great Britain and Ireland, residing at Rest Harrow, Gomshall, in the county of Surrey, England, have invented a new and useful Tanning Composition, of which the following is a specification.

This invention relates to an improved method of tanning hides which is particularly applicable for the production of sole leather, dressing leather and the like, and has for its object the efficient production of such material in a simple and certain manner and with a great saving of time compared with known methods.

The invention consists in the process of tanning treatment of hides as hereinafter described.

According to this invention the hides are treated by any ordinary process of depilation by the use of lime, sulfide and caustic soda. They are then fleshed and delimed in an acid bath or in old tanning liquor sufficiently acidified for the purpose.

The hides are now treated according to this invention by one or other alternative methods, viz., in a tanning drum or in tanning pits provided with agitating means, such as rockers or plungers.

Dealing with the treatment of hides for sole leather in the tanning drum first, for every 100 lbs. of hide the following solution is made. In two gallons of boiling water  $1\frac{1}{2}$  lbs. of hyposulphite of soda is dissolved to which is added 1 lb. of aluminum sulphate dissolved in as little boiling water as possible. Into this mixture is stirred  $\frac{1}{2}$  lb. of vaseline or equivalent mineral product

and 2 pints of glycerine or lanoline, the agitation of the whole being carried out to insure thorough mixture, which when effected is brought up to the boiling point, preferably by steam heat, but when such boiling point is reached, no further heat is applied. Half of this mixture is placed in the tanning drum, which is then filled with a liquor of  $30^{\circ}$  Barkometer, made with a tanning extract composed of myrobalan, gambier, quebracho, and mimoso, in practically equal proportions, and to the mixture so made, one quart of turpentine is added and thoroughly mixed therewith. The hides are now placed

in the drum and the latter is revolved at a slow rate of revolution for an hour when the other half of the first described mixture is added to the drum, which latter is run for four periods of six hours each with a rest of 2 hours every sixth hour, the strength of the tanning liquor being gradually increased to  $60^{\circ}$  Barkometer by the addition of said tanning extract, great care being taken that the strength of the solution is always slowly on the increase and that the temperature of the drum does not rise above  $100^{\circ}$  F. After the drumming operation the hides are removed from the drum and laid flat for one night and well sheeted. They are then placed in three rocker pits for 4 hours each in succession the pits containing a mixture of tanning extract and tanning liquor of  $90^{\circ}$ ,  $100^{\circ}$  and  $120^{\circ}$  Barkometer at a temperature of  $110^{\circ}$  F., said tanning liquor consisting of 25% myrobalan, 25% mimoso and 50% quebracho, chestnut or the like. After such treatment the hides are removed from the pits and are rinsed through acid liquor, piled for the night, oiled with a sulphonated oil and shedded in the ordinary way.

In dealing with the hides for sole leather by pit tannage the treatment is started with a mild liquor of  $20^{\circ}$  Barkometer, composed of 60% myrobalan, 20% gambier, and 20% quebracho, chestnut or the like, and if, for example, the pit is of 250 cubic feet capacity it is filled to about  $\frac{2}{3}$  with the above liquor. This liquor is heated, preferably by steam, to  $100^{\circ}$  F. and to it is added the following mixture:—

36 lbs. of hyposulphite of soda.

24 lbs. of aluminum sulphate.

12 lbs. of vaseline.

6 gallons of glycerine or lanoline and 2 quarts of turpentine.

During the addition of this mixture thorough agitation of the liquor is carried out in order to produce complete incorporation.

It is advisable to have rockers, plungers or other agitating means fixed in each pit and kept running for periods of 1, 2, 3, 4 and 5 hours, with a period of rest of 1 hour between each operation. After the hides have been rocked 24 hours including rests in the first pit they are placed in a second pit in

which the same chemical mixture is used, but of 30° Barkometer density. The hides are rocked in this pit for 3 hour periods with a rest of 1 hour between each for 6 hours, at 5 a temperature of 110° F. They are then transferred to the third pit with the same chemical mixture, but of 45° Barkometer density and are rocked at the same time and with the liquor at the same temperature as 10 in pit No. 2. They are then transferred to the fourth pit in which a chemical mixture of double the strength of the above is used, and of 75° Barkometer density at a temperature of 110° F. for a period of 12 hours. 15 No rocking takes place in this pit but the hides are handled twice over. They are then transferred to the fifth pit which contains liquor of 100° Barkometer at a temperature of 115° F. and are kept in the pit for 12 20 hours and rocked for periods of 3 hours with 1 hour's rest between each rocking. The hides are then finished in a similar manner to that described in the drum tannage.

In using the process for dressing leather 25 the above solutions should be of half the Barkometer density and half the proportion of chemicals as above indicated and the

process is carried out at normal atmospheric temperatures.

I claim:—

1. A composition for the tanning of hides, comprising hyposulphite of soda, aluminum sulphate, and vaseline in the approximate proportions by weight respectively of 1.5, 1 and .5, and a mixture of glycerine, tanning extract, and turpentine in the approximate proportions by measure respectively of 1, 35 2000, and 1.

2. A composition for the tanning of hides, comprising, for every 100 lbs. of hide, 1 $\frac{1}{2}$  lbs. 40 hyposulphite of soda, 1 lb. aluminum sulphate dissolved in 2 gallons of boiling water,  $\frac{1}{2}$  lb. vaseline, 2 pints glycerine, 500 gallons of a liquor of 30°-60° Barkometer made with tanning extract including myrobalan, gam- 45 bier, quebracho and mimosa in practically equal proportions, and 2 pints of turpentine.

In testimony whereof I have signed my name to this specification in the presence of two subscribing witnesses.

ROGER BUCHANAN COCK.

Witnesses:

WALTER CARVER,  
DORIS HITCHCOCK.